

# UNITED STATES PATENT OFFICE.

JAMES McINTOSH, OF NORRISTOWN, PENNSYLVANIA, ASSIGNOR TO DIAMOND STATE FIBRE COMPANY, OF BRIDGEPORT, PENNSYLVANIA, A CORPORATION OF DELAWARE.

## INSULATING MATERIAL AND PROCESS OF MAKING THE SAME.

1,267,883.

Specification of Letters Patent. Patented May 28, 1918.

No Drawing.

Application filed January 26, 1918. Serial No. 213,909.

*To all whom it may concern:*

Be it known that I, JAMES McINTOSH, a citizen of the United States, residing in Norristown, Montgomery county, Pennsylvania, have invented Insulating Materials and Processes of Making the Same, of which the following is a specification.

One object of my invention is to provide a substance which shall be hard, durable and waterproof, as well as possess other qualities fitting it for use as an electrical insulator, especially in connection with railway tracks.

I further desire to provide a simple, easily operated method of preparing the above noted material whereby it shall be possible to so treat vulcanized fiber as to render it more water-repellent and otherwise more suitable than hitherto for service as a track insulating material.

In carrying out my invention I employ as my chief raw material, vulcanized or parchmentized fiber in a green state;—that is to say, fiber in its finished condition except that it is saturated with water and has not been given the final drying or heat treatment ordinarily necessary to prepare it for commercial use. By my process, such green fiber is impregnated with an oxidizable oil, such as linseed oil or an equivalent substance, by replacing the water in it by an organic solvent such as acetone, by immersing it in a bath of the same, for a period of time dependent upon its thickness. For example, fiber sheets having a thickness of one-quarter of an inch have been found to require an immersion in the acetone bath of about forty-eight hours.

Thereafter the fiber is placed in a bath of linseed or other oxidizable oil for a similar period of time, as a result of which the solvent is replaced by said oil and the fiber is found to contain practically no water. The time and method of treatment may be varied by varying the temperature of the bath, by employing mechanical stirrers and by the use of a vacuum. In some cases the green fiber may be subjected to a vacuum while immersed in the oil, with the result that the contained water is removed and replaced to a greater or less extent by said oil.

In order to fit the oil-impregnated fiber resulting from the above treatment for use as a track insulation, which is usually required to have certain definite shapes, it is immersed in hot water or treated by live steam, as a result of which it becomes relatively pliable, so that it may be molded, bent or shaped by pressure, or heat and pressure. The oil is then slowly oxidized by heat treatment until it becomes semi-solid, such treatment usually requiring from twelve to thirty-six hours, depending on the thickness of the material.

As a result of this treatment the fiber is given a shape or form which it will permanently retain, and it is found to be hard, tough and practically waterproof, being incapable of absorbing appreciable amounts of water and not subject to injury by the weather. It is noted that the heat treatment oxidizes the oil so that it is changed to a solid gum, without in any way affecting the parchmentized fiber in which said oil is contained.

I claim;—

1. The process which consists in impregnating parchmentized fiber with an oleaginous body; treating said fiber to render it flexible; shaping the fiber to a definite form; and subjecting it to an oxidizing treatment to harden it and solidify said oleaginous material.

2. The method which consists in impregnating green parchmentized fiber with a substance capable of being solidified by heat; shaping the fiber to a predetermined form; and thereafter subjecting it to a heat treatment to solidify the substance therein.

3. The method which consists in impregnating parchmentized fiber with a water-repelling substance in liquid form; treating the fiber to render it flexible; giving the fiber a predetermined shape; and thereafter hardening it and solidifying the water-repelling substance therein.

4. As a new article of manufacture, a hard molded water-proof body consisting of parchmentized fiber uniformly impregnated with oxidized oil.

In witness whereof I affix my signature.  
JAMES McINTOSH.